

## UNITED STATES PATENT OFFICE

2,426,140

## NONSETTLING MINERAL FILLERS

Armand R. Bollaert, Palos Verdes, Calif., assignor  
to Great Lakes Carbon Corporation, a corpora-  
tion of Delaware

No Drawing. Application October 15, 1945,  
Serial No. 622,477

8 Claims. (Cl. 106—288)

1

This invention relates to the treatment of mineral filling agents to prevent them from settling from aqueous suspension in compact masses.

Many finely comminuted minerals used as filling or bodying agents in cold water paints and other aqueous suspensions show a tendency to settle out on standing for even brief periods. As a rule, a suspension of these substances, after standing undisturbed for a sufficient time, exhibits three distinguishable phases: an upper 10 layer of more or less clear water; an intermediate layer of slurry of variable consistency, and a hard and compact bottom layer. In extreme cases, as after long standing, the intermediate layer may be missing.

If the hard lower layer can be prevented from forming, the partial sedimentation which produces a concentrated slurry is harmless as this slurry, even if very thick, may readily be redispersed by simple stirring. The formation of a 20 hard layer, however, is highly objectionable. Such sediments, formed in a stored package, are tedious and difficult to again bring into suspension and are likely to result in lumping. Where such hard layers form in mixing vessels or tanks 25 the apparatus may have to be cleaned out before it can again be put into operation.

I have discovered that the formation of compact settled layers may be prevented, and sedimentation restricted to the formation of a thick 30 slurry, by mixing with the filler a small proportion of a highly colloidal clay, such as the so-called bentonite, together with a minute proportion of a salt of ammonium with a mineral acid. These admixtures do not prevent sedimentation 35 of the filler but, when used in suitable proportions, they maintain the settled layer in the soft and uncompacted condition in which it may readily be redispersed.

In order to determine the effectiveness of the 40 treatment, the optimum dosages of the agents and the specific ammonium salts most effective for the purpose, experiments were conducted with a diatomaceous earth filler consisting of the fines from the manufacture of high quality filter-aids by calcination with fluxing agents. This material settles rapidly from aqueous suspension to form hard layers which are very difficult to bring back into suspension.

In these experiments, 10 grams of the filler was dispersed in 100 ml. water, with or without the addition of one or more of the agents named in the table below. The suspensions were then allowed to stand undisturbed for eight days, after which an arbitrary measurement of the solidity of the settled layer was made by allowing a glass rod of  $\frac{1}{4}$ " diameter and weighing 46 grams to subside to constant level through it. As the diameters of the cylinders in which the tests were made varied slightly, the measurement made was of the per-

2

centage of the total volume occupied by the layer sufficiently solid to support the rod. As this figure is entirely arbitrary and useful only for comparison, numerous check experiments were made which showed that if this supporting volume did not exceed 14% of the total volume the settled layer could be redispersed without material difficulty, and that the difficulty experienced in redispersion increased as this percentage volume increased.

Ammonium chloride and Wyoming bentonite were added to this suspension in the proportions set forth below, with the following results:

15

Table 1

| Filler | Composition in Grams |          | Volume of Supporting Layer |
|--------|----------------------|----------|----------------------------|
|        | Bentonite            | Chloride |                            |
| 10     | 1.0                  | 0.10     | 0                          |
| 10     | 1.0                  | 0.06     | 11                         |
| 10     | 1.0                  | 0.05     | 16                         |
| 10     | 1.0                  | 0.04     | 16                         |
| 10     | 1.0                  | 0.03     | 18                         |
| 10     | 1.0                  | 0.02     | 18                         |
| 10     | 1.0                  | 0.00     | 18                         |
| 10     | 0.0                  | 0.00     | 21                         |
| 10     | 1.5                  | 0.06     | 0                          |
| 10     | 1.0                  | 0.06     | 11                         |
| 10     | 0.8                  | 0.06     | 21                         |
| 10     | 0.6                  | 0.06     | 21                         |
| 10     | 0.4                  | 0.06     | 21                         |
| 10     | 0.0                  | 0.06     | 21                         |

It will be noted that these percentage figures are good only for this particular filler and do not show the same critical limits when other fillers are substituted for diatomaceous earth.

When other ammonium salts were substituted for the chloride, in constant proportions, the following results were obtained:

15

Table 2

| Filler | Composition in Grams |      | Ammonium Salt Used | Volume of Supporting Layer |
|--------|----------------------|------|--------------------|----------------------------|
|        | Bentonite            | Salt |                    |                            |
| 10     | 1.0                  | 0.06 | Sulfate-----       | 0                          |
| 10     | 1.0                  | 0.06 | Chloride-----      | 11                         |
| 10     | 1.0                  | 0.06 | Phosphate-----     | 14                         |
| 10     | 1.0                  | 0.06 | Acetate-----       | 17                         |
| 10     | 1.0                  | 0.06 | Carbonate-----     | 19                         |
| 10     | 1.0                  | 0.06 | Oxalate-----       | 19                         |
| 10     | 1.0                  | 0.06 | Hydroxide-----     | 20                         |

The figures in these two tables show that neither bentonite alone nor the ammonium salt alone produce any material improvement in permanence and that they function together to produce the desired result. They also indicate a satisfactory stabilization of the suspension when the bentonite component is about 10% of the weight of filler taken and the ammonium chloride

about  $\frac{1}{10}$  of 1% of that weight. They also show perfect suspension when ammonium sulfate is substituted for the chloride in the above proportions, or when the proportion of chloride is raised to about 1% (with 10% bentonite) or when the proportion of bentonite is raised to about 15% (with 0.6% chloride). Finally, they indicate that satisfactory results are obtained only in the use of the ammonium salts of the strong mineral acids such as hydrochloric, sulfuric and phosphoric.

I claim as my invention:

1. A stabilized aqueous suspension of finely comminuted diatomaceous earth containing from 10 percent to 15 percent of a colloidal bentonite and from 0.6 percent to 1.0 percent of an ammonium salt of a strong mineral acid, said percentages being on the dry weight of earth in said suspension.

2. A stabilized aqueous suspension of finely comminuted diatomaceous earth containing from 10 percent to 15 percent of a colloidal bentonite and from 0.6 percent to 1.0 percent of ammonium chloride, said percentages being on the dry weight of earth in said suspension.

3. A stabilized aqueous suspension of finely comminuted diatomaceous earth containing from 10 percent to 15 percent of a colloidal bentonite and from 0.6 percent to 1.0 percent of ammonium sulfate, said percentages being on the dry weight of earth in said suspension.

4. A stabilized aqueous suspension of finely comminuted diatomaceous earth containing from 10 percent to 15 percent of a colloidal bentonite and from 0.6 percent to 1 percent of ammonium phosphate, said percentages being on the dry weight of earth in said suspension.

5. A mineral filling and bodying agent characterized by settling from aqueous suspension to form a soft and readily dispersible mass, consisting substantially of 100 parts of finely comminuted diatomaceous earth, from 10 parts to 15 parts of a colloidal bentonite, and from 0.6 part to 1 part of a salt of ammonium with a

strong mineral acid, all said parts being by dry weight.

5 6. A mineral filling and bodying agent characterized by settling from aqueous suspension to form a soft and readily dispersible mass, consisting substantially of 100 parts of finely comminuted diatomaceous earth, from 10 parts to 15 parts of a colloidal bentonite and from 0.6 part to 1 part of ammonium chloride, all said parts being by dry weight.

10 7. A mineral filling and bodying agent characterized by settling from aqueous suspension to form a soft and readily dispersible mass, consisting substantially of 100 parts of finely comminuted diatomaceous earth, from 10 parts to 15 parts of a colloidal bentonite and from 0.6 part to 1 part of ammonium sulfate, all said parts being by dry weight.

15 8. A mineral filling and bodying agent characterized by settling from aqueous suspension to form a soft and readily dispersible mass, consisting substantially of 100 parts of finely comminuted diatomaceous earth, from 10 parts to 15 parts of a colloidal bentonite and from 0.6 part to 1 part of ammonium phosphate, all said parts being by dry weight.

20 ARMAND R. BOLLAERT.

#### REFERENCES CITED

30 The following references are of record in the file of this patent:

#### UNITED STATES PATENTS

| Number       | Name        | Date          |
|--------------|-------------|---------------|
| 35 2,016,892 | Clarvoe     | Oct. 8, 1935  |
| 2,266,793    | Opperman    | Dec. 23, 1931 |
| 1,738,967    | Sadtier     | Dec. 10, 1929 |
| 1,758,145    | Clutterbuck | May 13, 1930  |
| 2,366,047    | Nerlinger   | Dec. 26, 1944 |

#### OTHER REFERENCES

Natural Mineral Paint Extenders, by Charles T. Harness.

National Paint Bulletin, June 1945, page 6.